

1,169,114.

E. O. BARSTOW,  
METHOD OF MANUFACTURING ARSENATE OF LEAD,  
APPLICATION FILED AUG. 1, 1912.

Patented Jan. 25, 1916.

2 SHEETS—SHEET 1.



WITNESSES=

Oliver M. Kappeler  
Shos. M. Say

INVENTOR—

Edwin O. Barstow  
BY Say and Oberlein  
ATTORNEYS—

E. O. BARSTOW.

METHOD OF MANUFACTURING ARSENATE OF LEAD.

APPLICATION FILED AUG. 1, 1912.

1,169,114.

Patented Jan. 25, 1916.

2 SHEETS—SHEET 2.



WITNESSES =

Oliver M. Kappeler

Thos. H. Fay

INVENTOR

Edward O. Barstow  
BY Fay and Oberlin  
ATTORNEYS

# UNITED STATES PATENT OFFICE.

EDWIN O. BARSTOW, OF MIDLAND, MICHIGAN, ASSIGNOR TO THE DOW CHEMICAL COMPANY, OF MIDLAND, MICHIGAN, A CORPORATION OF MICHIGAN.

## METHOD OF MANUFACTURING ARSENATE OF LEAD.

1,169,114.

Specification of Letters Patent.

Patented Jan. 25, 1916.

Application filed August 1, 1912. Serial No. 712,676.

To all whom it may concern:

Be it known that I, EDWIN O. BARSTOW, a citizen of the United States, and a resident of Midland, county of Midland, and State of Michigan, have invented a new and useful Improvement in Methods of Manufacturing Arsenate of Lead, of which the following is a specification, the principle of the invention being herein explained and the best mode in which I have contemplated applying that principle, so as to distinguish it from other inventions.

While the present invention is of principal interest in the manufacture on a commercial scale of lead arsenate, either the normal arsenate  $Pb_3(AsO_4)_2$  or the acid arsenate  $PbHAsO_4$ , the general mode of procedure, as well as the several specific methods or processes involved, are equally applicable to the manufacture of other insoluble arsenates than such lead arsenate, as for example, zinc, iron, and barium arsenates.

Said invention, then, consists of the steps hereinafter fully described and particularly pointed out in claims.

The annexed drawings and the following description set forth in detail various modes of carrying out the invention, such disclosed modes, however, constituting but several of the various ways in which the principle of the invention may be used.

In said annexed drawings: Figure 1 illustrates in diagrammatic fashion a typical apparatus such as may be employed in carrying on the various steps comprehended in the present improved process of manufacture; and Fig. 2 is a tabular exhibit of the different reactions which are assumed to occur in carrying on such process in the several modified ways hereinafter described.

The general method of procedure involved in the improved process under consideration consists in oxidizing an arsenic derivative to arsenic acid by means of a halogen, providing a compound to form a haloid with such halogen reagent, and adding a suitable compound of the metal, the arsenate of which is desired as a final product. As previously indicated, the process is applicable to any metal capable of being precipitated as such arsenate from its corresponding soluble salt, such as its haloid. Commenting further on this statement relative to the general mode of procedure, it

should be noted that it is immaterial, so far as the steps in the process are concerned, whether they be performed in the sequence just indicated, or in part, or in whole, simultaneously; and, as will be presently explained, the provision of a compound to go with the halogen reagent may, in a sense, be anticipated by adding the base employed for this purpose first, and oxidizing the arsenic derivative subsequently.

With regard to the several reactions exhibited in Fig. 2 of the drawings, it should be explained that these merely express the inventor's understanding of what takes place, and while they are believed to be indicative of the principal phenomena, and to properly explain the production of the end-products obtained, the actual process or processes hereinafter described, are not conditioned upon the actual occurrence of these reactions.

Reaction I. is intended to express what occurs when white arsenic or arsenious oxide ( $As_2O_3$ ), as the specific arsenic derivative of the general process previously outlined, is oxidized to arsenic acid by being treated with chlorin, as the specific halogen of such process, in the presence of water. There results a mixture of arsenic acid ( $H_3AsO_4$ ) and hydrochloric acid (HCl). To this acid solution an alkali, specifically sodium carbonate or soda ash ( $Na_2CO_3$ ) is then added in amount carrying base equivalent to the hydrochloric acid (HCl) contained in such solution. The solution thus obtained may, for convenience, be assumed to be arsenic acid and sodium chlorid or common salt ( $NaCl$ ), as per reaction III., but it is probable that arsenic acid, hydrochloric acid, sodium arsenate and sodium chlorid are all present, as well as free ions of sodium, chlorin and  $AsO_4$ . This same solution of arsenic acid and salt may be obtained by adding the alkali first, as has been already suggested is possible, and as is indicated in reaction II. of the tabular exhibit, Fig. 2. In this case the arsenious oxide is combined with soda ash, in the presence of water, and inasmuch as no carbonic acid gas is apparently evolved, the reaction is believed to be correctly represented as given. The exact intermediate phenomena are however immaterial here as in the other reactions; for on chlorinating the resulting solution, as represented by reaction IV., the

end result is the same as in the case of combining reactions I. and III., namely the equivalent of a solution of arsenic acid and common salt is obtained.

5 Instead of using soda ash, or equivalent alkali, in the fashion illustrated in reactions II. and III., sodium arsenate ( $\text{Na}_2\text{HAsO}_4$ ), or an equivalent soluble arsenate, may be used in quantity sufficient to furnish base 10 equivalent to the halogen used, in which case the arsenic acid contained in such soluble arsenate is liberated, the base uniting with the halogen to form a soluble haloid, as indicated by reaction XIV. Furthermore, a 15 solution assumed to be arsenic acid and a soluble chlorid, equivalent to that produced by reactions III. and IV., may be obtained by adding hydrochloric acid to a solution of a soluble arsenate, this reaction being shown 20 in equation XV. in which sodium arsenate solution is treated with hydrochloric acid. The solution from any of these reactions may accordingly be used in the remaining step of the process, which consists in reacting 25 with the solution thus obtained on a suitable compound of the metal of which the arsenate is desired. This remaining step, referring for the sake of illustration to the case where it is lead arsenate that is wanted, 30 is carried out by adding to the solution resulting from reactions III., IV., XIV. and XV., respectively, an oxid, hydrate, carbonate, or basic carbonate of lead, as per reaction V., which illustrates the use of the 35 oxid, and assumes the significant reagent in the solution to be arsenic acid. The result where each of the other lead compounds just referred to are employed is illustrated in the following reactions:—



As an alternative to the reactions given above to represent what happens when the arsenious oxid is chlorinated, the chlorin combined to form a chlorid, and an oxygen derivative of lead added to the resulting solution to form the desired arsenate, the following equations may be given:—



In other words, it is immaterial, so far as the reaction with the lead oxid is concerned, whether arsenic acid, or hydrochloric acid, or both, be assumed to be present; and in determining the amount of such oxid to be added, it suffices to determine the amount

of free acid present without inquiring as to which one it is.

The several preliminary reactions hereinbefore described may be conducted satisfactorily in suitable open tanks, or tubs, into 70 which the white arsenic and water in reaction I., or the white arsenic and soda ash and water in reaction II., are charged, as shown in Fig. 1; while the chlorination may be conducted in stone ware, coke-packed 75 chlorination towers, the mixture to be chlorinated being pumped continuously over said towers. In case reaction I. be followed 80 a stirrer may be fitted to the tank so as to keep the white arsenic in suspension in order that it will be pumped over the chlorinating tower together with the water; or the rate of pumping may be so great that enough arsenic will be carried in solution to take up the chlorin as fast as it is supplied, 85 and the tank itself be used simply as a saturating tank. In order to utilize all of the chlorin gas being furnished to the chlorinating towers in said reaction I. or in reaction IV., it has been found best to conduct 90 the chlorination in two steps or stages by providing two similar tank and tower units with independent pumps, the gas being passed in series first through the tower of unit No. 2 and then through the tower of 95 unit No. 1 and the raw materials being charged into the tank of the first unit and when partly chlorinated, being transferred to the second. This is the arrangement illustrated in Fig. 1, already referred to. The 100 charge in the first instance will in the meanwhile have been fully chlorinated and is forwarded to the next step in the process. This arrangement permits the complete absorption of the chlorin by the more active 105 raw materials, when commercial chlorin containing some air is utilized for the process, and also permits finishing the charge in the No. 1 unit without the escape of chlorin from the system. The lead oxid, or equivalent oxygen derivative, is then added to 110 the resulting solution of arsenic and hydrochloric acids, this operation being satisfactorily conducted in a wooden tank provided with a suitable stirrer, and with the solution so concentrated that the resulting mass will have the consistency of a cream, or paste. It has been discovered that by sufficiently prolonging the stirring, the lead arsenate may be made from the solid lead oxid, despite the fact that at first sight it 115 would seem that this reaction could not be carried to completion, because, the resulting product being solid, all of the lead oxid would not be reacted upon, but particles of it would be inclosed in an impervious coating of the lead arsenate. By subjecting the mixture, however, to prolonged stirring, or agitation, this tendency has been successfully overcome, as above indicated. 120

130

It has further been discovered that if, instead of adding an alkali, such as the sodium carbonate previously referred to, to the products resulting from reaction I., a suitable lead compound be added, such as the aforesaid lead oxid, hydrate, carbonate, or basic carbonate, there will be obtained a precipitate of lead chlorid and a solution of arsenic acid, as per reaction VI., such lead compound being added in amount sufficient to combine with the chlorin present. This reaction is accomplished in the same manner as that in which reaction V. is brought about; that is, the lead oxid, or 15 equivalent lead derivative, is mixed with the solution from reaction I. and stirred for a considerable length of time so that the lead oxid may become thoroughly converted to such lead chlorid, this operation being conducted in the presence of water insufficient 20 in amount to dissolve the lead chlorid that is formed. The solution of arsenic acid thus produced may then be separated from the solid lead chlorid, as by decantation or filtration, and used for the production of arsenate of lead by stirring with lead oxid, hydrate, carbonate, or basic carbonate, as in reaction 25 XIII., which illustrates the use of the oxid, or as in reaction X., which illustrates the use 30 of the carbonate. Again, instead of adding an alkali, (whether in the form of sodium carbonate as illustrated in reactions II. and III., or in the form of sodium arsenate as illustrated in reaction XIV.), simply in 35 quantity sufficient to furnish base equivalent to the halogen used, the acid solution resulting from reaction I. may be completely neutralized with alkali in order to produce the normal arsenate of lead instead of the 40 arsenate. The result of such neutralization, written for soda ash as the alkali, is exhibited in reaction XVI., the next step then being to stir lead chlorid (reaction XVII.) with the resulting solution with the production 45 of such normal arsenate of lead,  $Pb_3(AsO_4)_2$ .

It will thus be seen that the general process under discussion permits of the production of the acid arsenate of lead  $PbHAsO_4$ , or of the normal arsenate  $Pb_3(AsO_4)_2$ , in varying amounts, as may be desired, depending on how much of the original acid solution is deflected to the reactions III., VI., and XVI. It should further be explained 55 that preferably the lead oxid, hydrate, carbonate, or basic carbonate, where either of these is employed in the step resulting in the production of the arsenate, is not used in the proportions of its combining weight 60 with the arsenic acid present in the solution, but care is taken to not add sufficient lead compound to combine with all of such acid. It has been discovered that by proceeding in this way an arsenate higher in arsenic acid is obtained than if the materials be used in

the proportions of their combining weights. This is a distinct advantage in the production of commercial arsenates.

The lead chlorid used in reaction XVII. may be that separated out in reaction VI., 70 or it may be derived in any other suitable way. So, too, the chlorid thus resulting from the reaction last named may be employed in a further modification of the present general process by precipitating it as 75 lead carbonate, or hydrate, by treatment with soda ash, or lime. This step is shown, in reaction VIII., and the lead carbonate, or hydrate, so formed can be then used to produce lead arsenate by agitating with a 80 solution containing arsenic acid, as per equation X. the acid solution being produced by equation VI.; or such lead chlorid may be dissolved and precipitated as lead arsenate by reacting with a solution of a soluble arsenate as shown in equation XI., or otherwise 85 used as desired.

The exact compensation of the lead arsenate obtained in the reaction between lead chlorid and a soluble arsenate, as also its 90 physical properties, are dependent upon the ratio of base to arsenic in the arsenate solution. When sufficient base is present, normal arsenate  $Pb_3(AsO_4)_2$  is obtained, as per equation XII., in the form of a flocculent, 95 slow settling precipitate, and when less base is present, a mixture of the normal and acid arsenate  $PbHAsO_4$  is produced in the form of a granular rapid-settling precipitate. Equation XI., as written, shows one reaction 100 which occurs when not enough base is present to produce a normal arsenate.

Commercial sodium arsenate may be used to precipitate the lead arsenate, as above described, or a solution of a soluble arsenate 105 may be obtained by adding alkali to any of the various solutions of arsenic acid produced by the reactions above described. For instance, note reaction IX., in which the arsenic acid from VI. after being separated 110 as by filtration from the solid lead chlorid is neutralized with soda ash to produce a solution of sodium arsenate, which may then be utilized in carrying out the step exhibited in the reaction XII. just described. If, on 115 the other hand, the mixture of arsenic acid solution and lead chlorid resulting from said reaction VI. be treated as it stands with sodium carbonate, the acid lead arsenate may be produced in a single step as represented by the reaction of equation VII.

While the inventor prefers in some cases to separate the solid lead chlorid and to dissolve it before precipitating as lead arsenate, because in this way he is enabled to remove the insoluble impurities from the chlorid, which may have come from the use of an impure lead oxid and which would otherwise contaminate the final product, and further he is thereby enabled to obtain an arse-

- 5 nate having certain desirable physical qualities, yet he has discovered that the reactions given may be successfully conducted in the presence of water insufficient in amount to dissolve the lead chlorid, providing the mixture be stirred for a longer time than necessary where solutions are used, and if a pure oxid, carbonate or equivalent be used, there will be no impurities requiring separation.
- 10 This discovery enables him to conduct large scale operations of this nature in very much smaller tanks than if the lead chlorid, which is sparingly soluble, be dissolved, and a much larger output may be thereby obtained from a plant representing an equal investment. It would appear at first sight that such reactions could not be carried to completion because the resulting product, being solid, all of the lead chlorid would not be reacted upon but particles of it would be inclosed in an impervious coating of the lead arsenate. The inventor has successfully overcome this tendency, as above announced, by subjecting the mixture to prolonged stirring or agitation. This operation can be satisfactorily conducted in a wooden tank, provided with a suitable stirrer and with a solution so concentrated that the resulting mass will have the consistency of a thick cream. The inventor has further discovered that it is not necessary to separate the lead chlorid from the solution of arsenic acid, as obtained in reaction VI, but that arsenate of lead may be obtained directly by stirring the solid chlorid and arsenic acid solution with an alkali, as shown in reaction VII, and that in the presence of water insufficient to dissolve the lead chlorid and even in such concentration as to produce a mass having the consistency of cream. This step requires also prolonged stirring, as described for the similar reactions when using the lead chlorid separately, and if a pure lead oxid be used, a satisfactory arsenate may be obtained. This step, conducted with the solid chlorid and arsenic acid solution, has the same advantage of large output in small tanks, as already noted herein.
- 50 The oxygen derivatives of lead, which are suitable for use as compounds of that metal for reacting with arsenic acid to form lead arsenate, have been already indicated. The term "oxygen derivative" is intended therefore to connote such equivalents of lead oxid, or other lead compounds that have been specifically named, as will form the compound in question under the conditions surrounding the reaction. By way of general comment, it should further be noted that both the acid lead arsenate  $PbHAsO_4$ , and the normal arsenate,  $Pb_3(AsO_4)_2$ , are commonly known to the trade as arsenate of lead. The latter term is accordingly to be

understood as used in this general sense, 65 and not as referring specifically to either of the two arsenates named, except where the contrary is indicated.

It is proper to repeat, by way of conclusion, that the several equations of Fig. 2, 70 which have been referred to as expressive of the different reactions involved, are presented as illustrative merely of the principal phenomena. They do not, however, necessarily represent all of the reactions that occur, and should be understood as indicating how the desired end-product is derived rather than the exact intermediate steps leading up thereto.

From the standpoint of the manufacturer or practical chemist, it might be better to represent the whole series of detailed reactions pertaining to each particular process or sub-process described above, as a single comprehensive reaction, in which only the 85 starting materials and observed end-products are given. Thus, for example, the specific mode of operation herein claimed may be represented as follows:—



In other words, so far as the commercial operation of the process in hand is concerned, it may be regarded as consisting in 95 a reaction between white arsenic, chlorin, soda ash, and lead oxid. As has already been indicated the soda ash is typical of any suitable compound capable of combining with the chlorin, and may be lead oxid or 100 other oxygen derivative of lead.

Other modes of applying the principle of my invention may be employed instead of the one explained, change being made as regards the process herein disclosed, provided 105 the step or steps stated by any one of the following claims or the equivalent of such stated step or steps be employed.

I therefore particularly point out and distinctly claim as my invention:— 110

1. The method of making an insoluble metallic arsenate, which consists in reacting in the presence of water between arsenious oxid, a halogen, a compound to form a haloid with such halogen, and a compound of the 115 metal of which the arsenate is desired, such last-named compound being adapted to produce such arsenate upon being added to a solution of arsenic acid.

2. The method of making an insoluble 120 metallic arsenate, which consists in reacting in the presence of water between arsenious oxid, chlorin, a compound to form a chlorid with such chlorin, and a compound of the metal of which the arsenate is desired, such 125 last-named compound being adapted to produce such arsenate upon being added to a solution of arsenic acid.

3. The method of making an insoluble metallic arsenate, which consists in reacting in the presence of water between arsenious oxid, chlorin, an alkali, and a compound of the metal of which the arsenate is desired, such last-named compound being adapted to produce such arsenate upon being added to a solution of arsenic acid.

4. The method of making an insoluble metallic arsenate, which consists in reacting in the presence of water between arsenious oxid, chlorin, an alkali, and an oxid of the metal of which the arsenate is desired.

5. The method of making lead arsenate, which consists in reacting in the presence of water between arsenious oxid, a halogen, a compound to form a haloid with such halogen, and a lead compound, adapted to produce such arsenate upon being added to a solution of arsenic acid.

6. The method of making lead arsenate, which consists in reacting in the presence of water between arsenious oxid, chlorin, a compound to form a chlorid with such chlorin, and a lead compound adapted to produce such arsenate upon being added to a solution of arsenic acid.

7. The method of making lead arsenate, which consists in reacting in the presence of water between arsenious oxid, chlorin, an alkali, and an oxygen derivative of lead adapted to produce such arsenate upon being added to a solution of arsenic acid.

8. The method of making lead arsenate, which consists in reacting in the presence of water between arsenious oxid, chlorin, an alkali, and lead oxid.

9. The method of making lead arsenate, which consists in treating arsenious oxid with chlorin in the presence of water, thereby producing hydrochloric acid and arsenic acid; adding sodium carbonate in amount

substantially equivalent to such hydrochloric acid; and adding lead oxid.

10. In a method of making an insoluble metallic arsenate, the step which consists in reacting in the presence of water with arsenic acid on a suitable compound of the desired metal, the amount of such compound used being insufficient to combine with all the arsenic acid present.

11. In a method of making lead arsenate, the step which consists in reacting in the presence of water with arsenic acid on a suitable lead compound, the amount of such compound used being insufficient to combine with all the arsenic acid present.

12. In a method of making lead arsenate, the step which consists in reacting in the presence of water with arsenic acid on oxygen derivative of lead adapted to produce such arsenate therewith, the amount of such derivative used being insufficient to combine with all the arsenic acid present.

13. In a method of making arsenate, the step which consists in reacting in the presence of water with arsenic acid on lead oxid, the amount of such oxid used being insufficient to combine with all the arsenic acid present.

14. The method of making lead arsenate, which consists in treating arsenious oxid with chlorin in the presence of water, thereby producing hydrochloric acid and arsenic acid; adding sodium carbonate in amount substantially equivalent to such hydrochloric acid; and adding lead oxid in an amount insufficient to combine with all such arsenic acid.

Signed by me this 27 day of July, 1912. 80  
EDWIN O. BARSTOW.

Attested by—

A. N. PATRIARCH,  
LEO W. LOWE.